

# UNITED STATES PATENT OFFICE.

ERICK LUDVIG RINMAN, OF DJURSHOLM, SWEDEN.

## PROCESS OF RETTING FIBROUS SUBSTANCES.

1,344,719.

Specification of Letters Patent. Patented June 29, 1920.

No Drawing.

Application filed October 2, 1918. Serial No. 256,612.

*To all whom it may concern:*

Be it known that I, ERIK LUDVIG RINMAN, a subject of the King of Sweden, residing at Djursholm, in the Kingdom of Sweden, 5 have invented a new and useful Improvement in Processes of Retting Fibrous Substances, of which the following is a specification.

The present process of treating fibrous 10 substances is applicable to all such substances which contain fibers capable of being spun. Thus it is possible according to the present process in an advantageous and economical manner to treat not only such 15 fibrous substances which have heretofore been treated by retting, but also other fibrous substances for which there have hitherto not existed any suitable methods of retting.

It has already been proposed, for the purpose of retting, to treat the fibrous substances with a diluted solution of potassium 20 hydrate or sodium hydrate, but it has not been possible to use the fibers thus obtained 25 on account of the fibers being affected by the alkali used. According to the present invention a lye from a previous treatment of vegetable substances with the said alkalis to which lye the necessary quantity of free 30 alkali hydrate has been added, is always used as treating liquid, with or without the use of increased temperature and pressure. It has been found that the fibers obtained 35 in this manner become particularly good and serviceable, the presence of oxy compounds in such lyes reducing to a great extent the influence of the alkali on the fibers without preventing the extraction aimed at. Waste liquors having a specific gravity of 40 1.035 up to 1.1 may be used with advantage for producing a new treating liquid.

When the treating liquid has been removed by washing and after drying, if desired, the raw material thus treated is ready 45 to be subjected to the usual mechanical treatment for obtaining fibers capable of being spun. The process is most efficient if the treatment is made in a hot state. When the treatment is made in a hot state the most 50 suitable boiling liquid is a lye containing 0.2 to 2 per cent. by weight of sodium hydrate. The time of treatment may vary from one hour to a longer period. If the treatment is carried out at about 100° C. a 55 time of treatment of about 3 to 5 hours is required. If higher temperatures, for in-

stance 135° C., are used, the boiling time may be shortened to one to two hours. The use of artificial pressure also reduces the time of treatment.

During the treatment it is most advantageous to use lyes with a small percentage of alkali. This may of course be obtained in many ways. By allowing the treating liquid to pass from one treating receptacle to another, or by causing the liquid to circulate in other manner, it is possible to treat the raw material with a larger quantity of lye than that contained in the treating vessel. It is of course also possible during the treatment to supply the necessary alkali gradually to the boiling liquid in such manner that the liquid always contains the required quantity of free alkali hydrate.

The waste liquor obtained during these 75 treatments contains the alkali used and the extracted organic substances. In order to make the present process really economical it is necessary to recover the alkali used, and, simultaneously, the extracted organic 80 substances should be utilized for producing valuable products. This is preferably attained by dry distilling the waste liquors when suitably concentrated and mixed with the required quantity of strong bases, for 85 instance sodium hydrate and hydrate of lime, in the presence of superheated steam, preferably in the manner previously disclosed in respect of dry distillation of waste liquors from the sulfate cellulose manufacture. In this manner acetone, wood spirit, higher alcohols, ketones, oils, and a considerable quantity of wax, ammonia and amines are obtained. The recovered alkali 90 is used for preparing a new quantity of 95 treating liquid.

The following may be given as an example of the application of the present process to the retting of flax. Bundles of flax freed from the seeds are mounted in a 100 frame, preferably in vertical position. The frame with the flax is then introduced into the boiler, in which the flax is treated during about two hours at a temperature of about 135° C. with a waste liquor from a 105 previous boiling having a specific gravity of about 1.074 and containing about 0.2 to 1 per cent.  $\text{Na}_2\text{O}$ . A quantity of about 100 kg.  $\text{Na}_2\text{O}$  is consumed for each ton of air-dried flax, consequently, this quantity of 110 soda lye must be present in the boiling lye or be added to the same, together with an

excess quantity of about 10 per cent. After the boiling the lye is removed and washed away with water. The water remaining in the retted flax may preferably be first pressed out, the remaining water being evaporated by means of a current of hot air, or in other suitable manner.

I claim:

The process of retting fibrous substances which consists in treating the fibrous substances with a waste lye from a previous

treatment of vegetable substances with alkali hydrate to which waste lye free alkali hydrate has been added, and carrying out the treatment at a temperature of at least 90° 15 C. and with a treating liquid so concentrated that its specific gravity is at least 1.074 but the percentage of caustic alkali of which does not exceed 3 per cent. alkali hydrate.

ERIK LUDVIG RINMAN.